

Patented May 7, 1929.

1,711,733

## UNITED STATES PATENT OFFICE.

EDUARD HOUDREMONT, OF ESSEN, AND VICTOR EHMCKE, OF ESSEN-HUGEL, GERMANY, ASSIGNORS TO FRIED. KRUPP AKTIENGESELLSCHAFT, OF ESSEN-ON-THE-RUHR, GERMANY.

### STEEL ALLOY.

No Drawing. Application filed January 11, 1928, Serial No. 246,082, and in Germany January 28, 1927.

The invention has for its object to produce steel alloys which possess high strengths at high temperatures. This object is obtained according to the invention by the fact, that the steel alloy contains 8 to 18 per cent of chromium, 2 to 12 per cent of manganese, 3 to 12 per cent of tungsten, and up to 1 per cent of carbon.

Steel alloys have been proved to have quite particularly high strengths at high temperatures, which contain, besides the otherwise usual admixtures, 12 to 14 per cent of chromium, about 5 per cent of manganese, about 5 per cent of tungsten, and about 0.5 per cent of carbon.

What we claim and desire to secure by Letters Patent, is:—

1. A steel alloy consisting of 8 to 18 per cent of chromium, 2 to 12 per cent of manganese, 3 to 12 per cent of tungsten, and up to 1 per cent of carbon.

2. A steel alloy consisting of 12 to 14 per cent of chromium, about 5 per cent of manganese, about 5 per cent of tungsten, and about 0.5 per cent of carbon.

The foregoing specification signed at Cologne, Germany, this 19th day of December, 1927.

EDUARD HOUDREMONT.  
VICTOR EHMCKE.